

## UNITED STATES PATENT OFFICE.

FRED K. BEZZENBERGER, OF CLEVELAND HEIGHTS, OHIO, ASSIGNOR, BY MESNE ASSIGNMENTS, TO THE FULTON SYLPHON COMPANY, OF KNOXVILLE, TENNESSEE, A CORPORATION OF DELAWARE.

## FLEXIBLE METAL WALL AND METHOD OF MAKING SAME.

No Drawing.

Application filed July 26, 1924. Serial No. 728,375.

The present invention, relating, as indicated, to flexible metal walls and methods of making the same, is particularly directed to an improved method of making tubular corrugated flexible metal walls, which are commonly called bellows, of a metal which may be worked and formed in a soft condition and then tempered after the completion of the forming operations as distinguished from the methods which are now in use, all of which involve the tempering of the metal during the forming operations and either the subsequent removal of the temper, or the removal of the temper at one or more stages during the forming process. To the accomplishment of the foregoing and related ends, said invention, then, consists of the means hereinafter fully described and particularly pointed out in the claims.

The following description sets forth in detail one method and one product exemplifying my invention, such disclosed procedure and product constituting, however, but one of various applications of the principles of my invention.

Metallic bellows, such as are now generally used in thermostats, valves and similar articles are commonly made by one of two methods. In one method a tube is first drawn and is then successively corrugated by pressing the metal outward and inward from the original tube wall and then rolling these initially formed corrugations to deepen and narrow the same until the desired shape is finally produced. In this method it is necessary to anneal the partially formed bellows one or more times in the forming operations, since the pressing of the metal outwardly and inwardly sets up a considerable temper, particularly at the crests of the inner and outer corrugations, and unless this temper is reduced or removed the metal becomes extremely stiff and is very liable to breakage at this point in a subsequent operation.

Brass is almost invariably employed in the process named, and brass is tempered by being rolled, stretched or otherwise worked, the amount of temper being directly proportional to the amount of deformation of the metal so that practically any desired temper may be given a bellows when completed by varying the number of rolling operations and

the amount of deformation given to the metal subsequent to the last annealing operation.

The chief disadvantages of this method, which is the one in common use, are, first, that only a relatively soft metal, such as brass, is ordinarily employed because of the difficulty of rolling iron, steel, nickel or similar metals, and second, the number of separate operations which are required, there being usually not less than five separate rolling operations and usually one or more annealing operations. Another disadvantage is that the resulting bellows is not strong since it is formed of a relatively weak metal, namely, brass, and cannot be employed where high pressures are necessary unless either the thickness of the wall is made sufficiently great, which in most cases is not practicable because the bellows is then stiff and unresponsive in movement, or by using a two or three ply bellows.

A second method consists in expanding a tube by means of an internal fluid pressure to produce a complete fold or bellows in practically a single operation at a very great saving in time and with very much less breakage and loss than is usually met with in the method described above. The present method is a development of the fluid pressure method referred to above. I first draw a tube of either relatively pure iron, which may contain a small percentage of carbon, say .10%, or of some alloy of iron from which carbon is entirely absent. After being drawn, and if necessary at one or more stages of the several drawing operations, I anneal this tube so that when completely drawn it is in a soft or untempered condition. This soft tube is then expanded by fluid pressure introduced within it into spaced corrugations, as in the manner described in my Patent No. 1,506,966, granted Sept. 2, 1924, and this expansion of the tube into a bellows may be accomplished either in one or more expanding operations, all carried out by fluid pressure.

After the bellows is formed it may or may not be again annealed to place it in an untempered condition and the material of the bellows is then converted into steel by passing a carbon-carrying gas over the bellows for a considerable period. It is well

known that pure iron may be converted into steel or carbonized in this manner and that the carbon will penetrate a distance of about  $\frac{3}{2}$  of an inch into the iron exposed to the 5 carbon-carrying gas. As the ordinary bellows is but a few thousandths of an inch, usually from .005 to .012, the penetration is entirely sufficient to convert all of the metal of the bellows into steel.

10 The bellows may also be tempered by packing with a carbonaceous material, such as charcoal or any of the ordinary case hardening compounds, and after the cementation process, as this operation is ordinarily 15 termed, the bellows should be cooled in the furnace and then reheated to a temperature above the critical temperature of the metal, after which it should be quenched either in oil or water for the purpose of refining the 20 coarse structure which has resulted from the carbonizing treatment. In case carbon to the amount of about .75% has been induced in the metal the temperature should be maintained at about  $1380^{\circ}$  F., after which the 25 metal is re-heated to about  $750^{\circ}$  F., in order to draw and temper, and relieve the strain which has been set up.

By thus inducing the desired properties in the metal after the formation of the bellows, that is, by converting iron into steel 30 after the bellows has first been formed, I am able to use an inexpensive material and to give it an extremely high elasticity and tensile strength in the finished article. Thus 35 the metal of a steel bellows made by this method will have a tensile strength of about 125,000 pounds per square inch, while that of an ordinary brass bellows as now made has a tensile strength of not to exceed 65, 40 000 pounds, and are thus unfitted for many desirable uses for which my improved bellows is entirely adequate. It is essential in my new method to use a material into which the desired properties of elasticity and high 45 tensile strength may be induced after the final formation of the article, and so far as I now know, this limits the material

which may be used to pure iron or to iron alloys which can be converted into steel alloys in the manner described after the 50 bellows has been completely formed.

It will be understood that while I prefer to form the iron bellows by fluid pressure because of the economy of that process and the quality of the product, it may be 55 formed mechanically and in either case given the subsequent treatment described to convert the metal to steel.

Various alloys of iron may be similarly 60 treated for the purpose of inducing qualities into the finished bellows. Thus an alloy of iron with about  $3\frac{1}{2}$  to 5 per cent nickel lends itself readily to the carbonizing and subsequent treatments and produces a steel having markedly better qualities than those to 65 be found in a pure steel such as has been discussed above.

Other forms may be employed embodying 70 the features of my invention instead of the one here explained, change being made in 75 the form or construction, provided the elements stated by any of the following claims or the equivalent of such stated elements be employed, whether produced by my preferred method or by others embodying steps 75 equivalent to those stated in the following claims.

I therefore particularly point out and distinctly claim as my invention:

1. In a method of making flexible deeply 80 corrugated tubular metal walls, the steps which consist in forming a tube of soft ductile metal into a deeply corrugated tube, and then alloying with the metal of said tube a substance capable of increasing the 85 elastic limit and tensile strength thereof.

2. In a method of making a deeply corrugated steel bellows, the steps which consist in forming an iron tube into a deeply corrugated tube, and then converting the metal 90 of such tube into steel.

Signed by me, this 23rd day of July, 1924.

FRED K. BEZZENBERGER.